

Feb. 26, 1957

B. B. RANEY

2,783,196

METHOD OF PRODUCING TITANIUM AND ZIRCONIUM

Filed March 19, 1952



INVENTOR

*Ben B. Raney*

BY *Pierce, Schaffer & Parker*

*Assoc. ATTORNEYS*

1

2,783,196

## METHOD FOR PRODUCING TITANIUM AND ZIRCONIUM

Ben B. Raney, Linton, Ind., assignor to Chicago Development Corporation of Delaware, Riverdale, Md.

Application March 19, 1952, Serial No. 277,445

1 Claim. (Cl. 204—64)

This invention relates to the production of the metals, titanium and zirconium. It has for its object the production of such metals substantially free from oxygen.

In my copending applications, Serial No. 230,336, filed June 7, 1951; Serial No. 256,385, filed November 14, 1951 and Serial No. 152,175 filed March 27, 1950, I have disclosed methods which are applicable to the production of titanium and zirconium, and this application may be considered a continuation in part of these applications. In my application, Ser. No. 152,175, filed March 27, 1950, I have disclosed the reduction of titanium halides by nascent alkali or alkaline earth metals formed at the cathode in the electrolysis of halides of these metals. In my application, Serial No. 230,336, filed June 7, 1951, I have disclosed the chlorination of titanium containing oxygen at an anode in an electrolytic cell and the reduction of the chloride so formed, by a solution of alkali or alkaline earth metal in a halide of these metals, which is formed at the cathode in such a cell. In my copending application Serial No. 256,385, filed November 14, 1951, I have disclosed reduction of metal compounds in situ by a solution of alkali or alkaline earth metal in a molten chloride of such metals.

In the present application, I disclose the formation of chlorides of titanium and zirconium by the anodic chlorination of titaniferous or zirconiferous oxygen-containing metal according to the equation as illustrated for titanium:



This reaction takes place at the anode in a molten bath of alkali or alkaline earth metal chlorides.

The present application discloses a separation of the  $\text{TiO}_2$  or  $\text{ZrO}_2$  formed, from the solution of  $\text{TiCl}_2$  or  $\text{ZrCl}_2$  in the molten chlorides. This separation is not disclosed in my copending applications.

Finally, the present application discloses a new combination of steps to produce pure metals from oxygen-containing material and apparatus for carrying out these steps.

My present invention consists in carrying out at least some of the following steps, illustrated for titanium:

(1) The reduction of titaniferous oxygen-containing material to a metallic alloy.

(2) The chlorination of the titanium-oxygen combination at the anode in an electrolytic cell in the presence of a bath of molten metallic chlorides containing at least one alkali or alkaline earth chloride with an amount of chlorinating agent not in excess of that necessary to form  $\text{TiCl}_2$  and  $\text{TiO}_2$  from the titanium present whereby to form a solution of  $\text{TiCl}_2$  in the molten chloride bath.

(3) Separating the solution of  $\text{TiCl}_2$  in the molten chloride bath from the insoluble residue.

(4) Reducing the  $\text{TiCl}_2$  in the molten chloride bath to metallic titanium at the cathode.

(5) Separating the titanium from the fused salts, and returning the fused salts to the second step.

Each of these steps may be carried out in various ways. The starting compound of titanium and oxygen may, for

2

example, be titanium metal scrap, containing oxygen. It is preferable that the raw material contain no chlorinatable material other than the titanium compound. Otherwise, provision must be made to remove such impurity in the third step of the process, in order to avoid contamination of the titanium metal produced. The  $\text{TiO}_2$  which is obtained as a residue from the chlorination step may be purified and reduced, for example, by heating with carbon. The chlorination step may be carried on by including the titanium-oxygen combination to be chlorinated in a conducting electrode which is made an anode in the fused chloride bath. This procedure provides a suitable excess of the titanium to be chlorinated. The molten chloride may be a single salt, such as  $\text{LiCl}$ , or it may be a mixture of alkali or alkaline earth metal chlorides. For the purposes of this description, magnesium is considered an alkaline earth metal. The separation of the fused chloride containing  $\text{TiCl}_2$  may be made, for example, by hot filtration through a bed of broken solids, or by means of a centrifuge. If separation is accomplished by a bed of broken solids, at least part of such bed may be metallic titanium. This titanium will react with, and remove the metals which may have been chlorinated from the raw material, and which are more readily reduced than titanium. Iron is an example of an impurity which may be removed in this way. The reduction of the  $\text{TiCl}_2$  by an alkali or alkaline earth metal is accomplished when anodic chlorination is used, by introducing a cathode into the fused salt containing  $\text{TiCl}_2$ , and which has been separated from the insoluble residue. In this procedure, it is of course necessary that the fused salt electrolytic bath be continuous from step 2 through step 4. The separation of the metallic titanium from the fused salt may be accomplished by filtering or centrifuging. The metal-free fused salt so recovered may be returned to step 2. The separated titanium may be freed from the last traces of salt by washing with water. In certain instances, the titanium metal may be recovered in massive, rather than particulate form, and its separation may therefore be greatly simplified.

The temperature for carrying out my invention is not critical. It may be anywhere above the melting point of the salt bath, but below the temperature at which volatilization becomes objectionable. In general, I prefer salt mixtures which can be used in the range 600–800° C.

In the above and further description of my process herein, I sometimes discuss only titanium. My process is applicable to zirconium, using the identical steps.

In carrying out my process as described, I prevent contact of the fused salt with oxygen or water vapor. This may be done by maintaining the apparatus completely filled with salt, or by providing an inert atmosphere.

In one embodiment of my invention a fused salt is fed into an anode compartment of an electrolytic cell and made to flow around the anode rapidly and through a filter into a compartment containing an inert conducting cathode, for example iron or graphite, a solution of alkali or alkaline earth metal in the fused salt is formed at this cathode and is admixed with the fused salt flowing through the filter to produce the finely divided metal dispersed through the salt in this compartment. The salt and dispersed metal may be removed from this compartment periodically and the metal recovered by dissolving the salt in water.

In order to make my process substantially continuous, I pass the fused salt from the cathode compartment through a filter and return the solid-free salt to the anode compartment.

The function of this second filter is to remove the metal particles from the bath and to avoid contamination of these particles the filter may be composed of somewhat larger particles of the same metal which may be recovered

for re-use by screening on a size basis or iron particles may be used and separated magnetically. The metal particles formed in the bath may be themselves used as a filter bed if the bath is allowed to settle somewhat to form such a bed. The filtrate cake formed in this way is not contaminated with other material. It may be conveniently separated and pressed under 10-50 tons/sq. in. at a temperature where the salt is molten to remove the salts and consolidate it into solid metal. This solid metal is ready to fabricate.

In the figure, I have illustrated an apparatus for carrying out my invention. It consists of a ceramic cell which is heated to a temperature necessary to melt the chlorides. The means for maintaining such temperature are not illustrated in the figure, but are conventional for maintaining molten salts in ceramic chambers as for the heat treatment of metal parts. Referring to the figure, the chamber A is separated from the remainder of the cell by a perforated partition. The chamber A is also connected by the large conduit, K, with chamber F which is likewise separated from the remainder of the cell by a perforated partition. The chamber F is provided with a pump I, so arranged as to circulate the fused salts into the chamber F from the remainder of the cell, and out through the conduit K, and thence into chamber A to be again drawn through the cell. The chamber B is provided with the anodes G. These anodes are made from the titaniferous oxygen-containing material, from which the metal is to be made. They may be made conducting by the addition of graphite. The fused salts are forced through the perforated partition from chamber A around the anodes G, in chamber B, and thence through a bed of filter material C. This filter material is held between two perforated partitions. It may be removed periodically through outlet J<sub>1</sub> in the bottom of the cell. New filter material may be filled in at the top. The action of the pump I forces the fused salts through the filter C, and into the cathode chamber D. In the cathode chamber, there are several cathodes H, between which the filtered fused salts pass. After passing between the cathodes H, the fused salts contain reduced metal. This reduced metal is removed in filter E, which is retained between two perforated partitions. The material of filter E may be discharged through the outlet J<sub>2</sub>, and new filter material supplied at the top. The metal is recovered from the filter material. The fused salts after removal of the metal by filter E are returned to chamber F, from which they are re-circulated through the cell. The cell is provided with a tight fitting cover, not shown in the figure, and a neutral atmosphere is maintained in the cell, above the fused salts.

The temperature for the practice of my invention depends on the anode material and the salts used. The temperature is preferably from 50-100° C. above the melting point of the salts and is limited as to high temperature only by excessive volatilization of the salt; with anodes composed essentially of the metals, temperatures as low as 450° C. may be used.

The current density at the anode should be at least 150 amperes/sq. ft. and the voltage at least 2.0. In the interest of economy, much higher current densities will be used and voltages up to 9.0 volts. The upper limit of current density will be determined by excessive heating and volatilization of the bath.

Having now described my invention in its general aspects, I will illustrate it by the following examples:

#### Example I

To carry out the procedure of this example, I make use of an apparatus like that in the drawing. The apparatus is completely filled with a molten bath of KCl and CaCl<sub>2</sub> freed from oxygen. The entire apparatus is maintained at 750° C. The anodes used are titanium scrap containing oxygen. The filter between the anode and cathode compartments is a bed of fine quartz particles, and the filter between the cathode compartment and the pump compartment is titanium particles. In carrying out this

example, the pump is operated at such a rate that precipitation of the titanium particles takes place at the entrance of the cathode compartment. That is, reduction takes place by a solution of calcium in the fused chlorides. 5 The material in the filters is periodically replaced by adding the filter bed material at the top, and withdrawing the material at the bottom. The metallic titanium from the second filter is freed from salt by washing with water.

#### Example II

10 In Example II, I proceed exactly as in Example I, except that the rate of operation of the pump is so regulated that less than all of the titanium chloride in solution in the salt is reduced to titanium metal during passage 15 through the cathode compartment. Titanium metal is deposited on the cathode by reduction of a portion of the chloride. In order to insure this excess at the start of the operation, I add a small amount of chlorine at the anode. By careful regulation of the rate of flow of the 20 electrolyte, a very slight excess of TiCl<sub>2</sub> can be maintained in the cathode compartment with only very small and infrequent additions of chlorine at the anode. When the cell is operated with an excess of TiCl<sub>2</sub> in the cathode compartment the titanium metal is deposited on the cathodes, and may be removed with them. Adhering salt 25 may be readily washed off.

#### Example III

I proceed as in Example II and when the relatively 30 massive metal is formed on the cathodes I press it to the bottom of the chamber where it accumulates as a mass of metal intermixed with some fused salt. I remove this mass from the bath and press it at 25 tons/sq. in. at 750° C. The salts are forced out of the metal and a solid 35 workable piece of metal obtained.

#### Example IV

I proceed as in Example I except that I prepare the 40 anode from a titanium oxide containing less oxygen than TiO<sub>2</sub>, and metallic titanium. The proportions used are such that the resulting product is a solid solution of oxygen in metallic titanium. Such solid solutions are 45 electrically conducting and may be used as anodes without contamination of the melt with carbon. The limit of these solid solutions is about 13% oxygen. The titanium used may be scrap or some of the product of the process used as a circulating load. The metal and oxide are heated to 800-1000° C. in the absence of air to produce a sintered product for use as anode. The TiO<sub>2</sub> 50 which is formed from the oxygen in the anode is separated from the anolyte by filtration as in Example I.

What is claimed is:

Process of producing substantially pure titanium from 55 crude titanium metal containing oxygen in solid solution, which comprises making the oxygen-containing titanium metal the anode in an electrolytic cell having communicating anode and cathode zones and means for preventing passage of particulate solids from one to the other of said zones, said cell being provided with a conducting cathode and with an electrolyte composed of at least one alkalinous metal chloride free from oxygen and with a protective inert atmosphere above said electrolyte, maintaining the cell contents at a temperature from 50 to 100° C. 60 above the melting point of the alkalinous metal chloride, continuously moving electrolyte from the anode zone to the cathode zone and over said cathode, passing a unidirectional current between anode and cathode at a current density of at least 150 amperes per square inch of anode surface and at an impressed voltage of from 2 to 9 65 volts, whereby to form in the electrolyte, in said anode zone, a solution of titanium di-chloride and particulate titanium dioxide, adding chlorine adjacent the anode, separating solid residue comprising said particulate titanium dioxide from said solution, passing the solution into the 70 cathode zone and over said cathode, the amount of chlo- 75

rine added being such, and said solution being passed over said cathode at such a rate, as to provide that the electrolyte after passing over the cathode contains a significant content of titanium di-chloride, thereby depositing pure titanium metal on the cathode sufficiently adherent to the latter that the deposit may be removed with the cathode, and removing associated electrolyte from such deposit.

## References Cited in the file of this patent

## UNITED STATES PATENTS

10

|           |                     |               |
|-----------|---------------------|---------------|
| 1,861,625 | Driggs et al. ----- | June 7, 1932  |
| 2,205,854 | Kroll -----         | June 25, 1940 |
| 2,413,411 | Kroll -----         | Dec. 31, 1946 |
| 2,550,447 | Blumenthal -----    | Apr. 24, 1951 |
| 2,564,337 | Maddex -----        | Aug. 14, 1951 |

15

|           |                        |               |
|-----------|------------------------|---------------|
| 2,607,674 | Winter -----           | Aug. 19, 1952 |
| 2,616,784 | Reimert -----          | Nov. 4, 1952  |
| 2,622,005 | Aagaard et al. -----   | Dec. 16, 1952 |
| 2,707,169 | Steinberg et al. ----- | Apr. 26, 1955 |

|         |                     |              |
|---------|---------------------|--------------|
| 635,267 | Great Britain ----- | Apr. 5, 1950 |
| 253,055 | Switzerland -----   | Nov. 1, 1948 |
| 553,056 | Great Britain ----- | May 6, 1943  |

## FOREIGN PATENTS

|                                                                                                                     |
|---------------------------------------------------------------------------------------------------------------------|
| “Chapters in the Chemistry of the Less Familiar Elements,” by Hopkins, vol. 1, chap. 11, page 7, published in 1939. |
| “Transactions of The Electrochemical Society,” vol. 87 (1945), pages 551 thru 567, article by Kroll.                |

## OTHER REFERENCES